

1,387,425.

M. M. MERRITT,  
ELECTROLYTIC PROCESS AND APPARATUS.  
APPLICATION FILED OCT. 13, 1919.

APPLICATION FILED OCT. 13, 1919.

Patented Aug. 9, 1921.

2 SHEETS—SHEET 1.



*Inventor:*  
Matthew M. Merritt,  
by Emery Booth Jameson Varney,  
Attys.

M. M. MERRITT,  
ELECTROLYTIC PROCESS AND APPARATUS,  
APPLICATION FILED OCT. 13, 1919.

1,387,425.

Patented Aug. 9, 1921.

2 SHEETS—SHEET 2.

Fig. 2.



Fig. 4.



Fig. 3.



Inventor:

Matthew M. Merritt,  
by Emery Booth Jenney & Varney  
Atty's.

# UNITED STATES PATENT OFFICE.

MATTHEW M. MERRITT, OF SOUTH MIDDLETON, MASSACHUSETTS, ASSIGNOR TO  
MERRITT METALS COMPANY, OF SALEM, MASSACHUSETTS, A CORPORATION  
OF MAINE.

## ELECTROLYTIC PROCESS AND APPARATUS.

1,387,425.

Specification of Letters Patent.

Patented Aug. 9, 1921.

Application filed October 13, 1919. Serial No. 330,403.

To all whom it may concern:

Be it known that I, MATTHEW M. MERRITT, a citizen of the United States, and a resident of South Middleton, county of Essex, State 5 of Massachusetts, have invented an Improvement in Electrolytic Processes and Apparatus, of which the following description, in connection with the accompanying drawings, is a specification, like characters on the 10 drawings representing like parts.

This invention pertains to improvements in electrolytic processes and apparatus.

In the drawings, which show an illustrative embodiment of a preferred form of apparatus with which my improved method 15 may be practised:—

Figure 1 is a side elevation, partly in section;

Fig. 2 is a plane view;

Fig. 3 is a section on the line 3—3 of Fig. 20 1; and

Fig. 4 is a detail view showing one form 25 of rack for supporting cathodes which may be used in connection with my invention.

In the preferred form shown in the drawings I have provided a tank 5 containing a supply of electrolyte 6 which may be pumped therefrom by a centrifugal pump 7 and discharged through a pipe 8 into an inclined trough 9 down which the electrolyte 30 may flow between anodes 10 past the cathode or cathodes 11 into a second inclined trough 12 also preferably containing anodes and cathodes, which trough returns the electrolyte to the tank 5, preferably providing for 35 aeration of the electrolyte by providing a fall 13 which preferably supplements an initial fall 14 where the pipe 8 discharges into the first inclined trough 9.

I have elected to show the anodes 10 as 40 bodies of relatively small pieces of metal, preferably copper, confined behind screens 15 which are preferably located relatively close to the cathodes 11. I have also elected 45 to show my improved apparatus and process as used in connection with the manufacture of tubes for aeroplane or other radiators, the tubes being clamped between non-conductive strips 16—16, preferably of wood, and bored 50 at intervals to receive the ends of the tubes. I have shown an electric connection to these cathodes through a wire 17 passing along one of the non-conductive strips. The connection to the anodes may be made in any 55 suitable way, as by plates 18 passing down

the sides of the troughs. The amount of space between the anodes 10 and cathodes 11 is preferably such that, taking into consideration the slope of the troughs, the electrolyte will pass down the troughs at a relatively high rate of flow while maintaining a substantially constant depth. I may, if desired, provide gates 19 to regulate or control to some extent the rate of flow. The depth and rate of the flow is also, of course, to some extent controlled by the rate at which the centrifugal pump circulates the electrolyte. Where an acid electrolyte is used the centrifugal pump, pipe, etc., should be lined with lead or other material not affected by the acid.

My improved process may be practised with the before-described apparatus or any other suitable apparatus, and preferably comprises electro-deposition on cathode material while the electrolyte flows past the cathode. It also preferably comprises the use of cathodes in the flowing stream of electrolyte so that the ionic supply from the cathode to the electrolyte is constantly renewed in various parts of the flowing stream. It also preferably includes the location of the anode material in close proximity to the cathode material and, where a plurality of cathodes are used, the distribution thereof longitudinally of the stream. As a matter of economy, my process preferably includes the circulation of the electrolyte so that it is used again and again. I have found that aeration of the electrolyte 50 in any suitable way, but preferably by providing one or more falls in the circulatory system, is of marked advantage in ridding the electrolyte of occluded hydrogen, and seems to otherwise increase the efficiency 55 thereof. I have found that the use of the swiftly flowing stream of electrolyte enables me to utilize a much higher current density per square foot of anode surface than could otherwise be used without impairing the 60 quality of the deposited material and that the constant renewal of the ionic supply to the electrolyte in the flowing stream, preferably coupled with proximity of cathode material to the anode material, promotes evenness of deposit throughout the 65 cathode surface area in different portions of the stream.

While I have shown and described apparatus which constitutes a preferred embodiment 70

ment of my invention, and while I have described a preferred way of practising my improved method, it will be understood that changes in the apparatus and even changes 5 in the method described may be made without departing from the scope of my invention, which is best defined in the following claims.

Claims:

- 10 1. Apparatus for use in electro-deposition comprising means for holding a plurality of objects distributed longitudinally of a flowing stream of electrolyte, negative electrical connections to said objects to render 15 the same cathodes, and anodes distributed lengthwise of the stream adjacent said cathodes.
- 20 2. Apparatus for use in the electro-deposition of tubes comprising holders for the tube cores, a trough in which said holders and the tube cores held thereby may be held, negative electrical connections to said cores rendering the same cathodes, anode material distributed lengthwise of said trough and 25 means for rapidly circulating an electrolyte through said trough.

3. The method of electro-depositing metal on a plurality of relatively small separate objects which comprises holding said objects in spaced relation in a stream of rapidly flowing electrolyte, while said objects are rendered cathodes by connection to a negative electric pole, and while anodes are distributed lengthwise of the stream adjacent the cathodes. 30

4. The method of forming tubes by electrolysis which comprises holding the tube mandrels in spaced relation in a flowing stream of electrolyte while an end of the tube is in contact with a negative electric 35 conductor.

5. The method of electro-depositing metal on a plurality of separate objects which comprises immersing said objects in a stream of rapidly flowing electrolyte, while said objects are rendered cathodes by connection to a negative electric pole, and while anode material is immersed in the stream adjacent 40 said cathodes.

In testimony whereof, I have signed my 45 name to this specification.

MATTHEW M. MERRITT.